

## UNITED STATES PATENT OFFICE

CHARLES SAMUEL BEDFORD, OF LEEDS, ENGLAND

## PROCESS FOR MORDANTING AND DYEING OF WOOL

No Drawing. Application filed January 15, 1926, Serial No. 81,589, and in Great Britain April 23, 1925.

This invention relates to processes for mordanting wool and has for its object an improved process for mordanting wool with chromium salts.

According to this invention I perform the mordanting of wool with chromium salts in such a manner as to effect the total reduction of the bichromate employed to the state of chromium hydroxide. In this form the mordant gives the fastest shades to light, milling and potting with colouring matters capable of being dyed on chrome mordant, and in most cases the shades produced are brighter and more intense than when the ordinary processes of mordanting are employed.

As a reducer of bichromate in presence of the wool I employ the salts of thiosulphuric acid, preferably on account of cost—the sodium salt, sodium thiosulphate, sometimes termed sodium hyposulphite.

When this salt is acted upon by dilute acids it decomposes yielding sulphur (at first in the colloidal state) and sulphurous acid. These substances exert a reducing action on the bichromate, being in turn oxidized to sulphuric acid. Sulphites or bisulphites cannot be employed instead of the thiosulphates in my process. At the boiling temperature they are uncontrollable and too energetic in their action, so that irregular and uneven results are obtained. For the purposes of my invention a thiosulphate must be used.

In mordanting wool I proceed according to one of the two following methods:—

## Example 1

For 500 lbs. loose wool in a dyeing machine through which hot water is circulating I add 10 lbs. of bichromate of soda in strong solution whilst the mordant bath is at 60° C. or thereabouts. Circulation is continued and the temperature gradually raised. After 20 minutes and whilst the temperature is about 90° to 93° C. I add gradually 15 lbs. sulphuric acid diluted with water. Boiling is continued for further 20 minutes, then I add gradually a solution of 5 lbs. sodium thiosulphate. After 30 minutes further boiling the bath will be found to be free from chrome salts.

In order to render the action of the thiosulphate more certain, and to prevent any risk of sulphur being deposited, I find it is beneficial to add to the mordanting bath along with the thiosulphate  $\frac{1}{4}$  to  $\frac{1}{2}\%$  of borax on the weight of the wool, or  $\frac{1}{2}$  to 1% of sodium acetate. These additions certainly enable the mordanting to be performed with greater regularity and in less time.

## Example 2

For 500 lbs. of woolen cloth in a dyeing machine I add 10 lbs. bichromate of soda in strong solution whilst the bath is at 60° C., and with the winch running. The temperature is gradually raised to 90° to 95° C. and after 20 minutes I add gradually during 30 minutes  $15\frac{1}{2}$  lbs. sulphuric acid diluted with water. An addition of 5 to  $5\frac{1}{2}$  lbs. sodium thiosulphate, and  $1\frac{1}{4}$  to  $2\frac{1}{2}$  lbs. of borax is then made, and the boiling continued until all chrome is fixed on the fibre.  $2\frac{1}{2}$  to 5 lbs. of sodium acetate may be substituted for borax.

The mordant thus fixed is sufficiently basic for most purposes of dyeing, but when chromium hydrate only is required the small proportion of acid groups in combination with the hydrate must be neutralized by an alkali.

In order to produce the pure chromium hydroxide mordant, the wool prepared as above is then treated in the same or in a separate bath at 60° to 93° C. with an addition of mild alkali such as sodium carbonate or ammonia sufficient to bring about a neutral condition when it is ready for dyeing. The dyeing may be conducted in the same ("sequence dyeing") or in a separate bath.

In most cases the dyeing can be started at once by addition of the dye to the hot neutral or slightly alkaline bath, when in the case of hematine the colouring matter will commence dyeing the fibre, in other cases the addition of a weak acid is necessary to start the dyeing. As a simplification I mix sodium carbonate with the dye to be used, in quantity sufficient to render the bath slightly alkaline after addition, and when the hydroxide mordant has been properly

formed I gradually add acetic, lactic or formic acid to give an acid reaction to the dyebath.

5 My invention includes the dyeing of the wool which can follow the mordanting in the same vessel in sequence, with consequent saving in steam, labour and time.

10 "Sequence dyeing" is found extremely useful for compound blacks using hematine along with such fast blacks as Durachrome Black A, Eriochrome Blacks A & T, and Diamond Black P. V.

15 Diamond Black P. V. is however an after-chrome colour, and in using it and other after-chrome colours I proceed as follows:—

20 The wool is first dyed with say 4% of colouring material and 2% concentrated sulphuric acid containing 96%  $H_2SO_4$ . When the exhaustion is complete 2% bichromate of 25 soda is added and boiling is continued for further 40 minutes, then 2% of concentrated sulphuric acid containing 96%  $H_2SO_4$  followed by 1% thiosulphate are gradually added, and the boiling continued until the 30 bath is exhausted of chrome salts. 4% hematine crystals containing 10% sodium carbonate are then added, and finally towards the end of the dyeing sufficient acetic acid to give an acid reaction.

35 30. What I claim and desire to secure by Letters Patent is:—

1. A process for chrome mordanting wool so that all the chrome is withdrawn from the mordanting bath and fixed upon the wool, 35 leaving the bath fit for use in a dyeing operation by treating the wool in a boiling bath with a bichromate and sodium thiosulphate and a mild alkali as a regularizing agent in the presence of a little acid.

40 2. A process for chrome mordanting wool so that all the chrome is withdrawn from the mordanting bath and fixed upon the wool, leaving the bath fit for use in a dyeing operation by treating the wool in a boiling bath 45 with a bichromate and sodium thiosulphate and borax in the presence of a little acid.

3. A process for chrome mordanting wool so that all the chrome is withdrawn from the mordanting bath and fixed upon the wool, 50 leaving the bath fit for use in a dyeing operation by treating the wool in a boiling bath with a bichromate and sodium thiosulphate and borax in the presence of a little acid.

4. A process for chrome mordanting wool 55 so that all the chrome is withdrawn from the mordanting bath and fixed upon the wool, leaving the bath fit for use in a dyeing operation by treating the wool in a boiling bath with a bichromate and sodium thiosulphate and borax in the presence of a little acid, and 60 then dyeing the wool with a mordant dyeing color.

5. A process for chrome mordanting wool so that all the chrome is withdrawn from the 65 mordanting bath and fixed upon the wool,

leaving the bath fit for use in a dyeing operation by treating the wool in a boiling bath with a bichromate and sodium thiosulphate and borax in the presence of a little acid, and then dyeing the wool with a mordant dyeing 70 color in the same bath.

In testimony whereof, I affix my signature  
CHARLES SAMUEL BEDFORD.

75

80

85

90

95

100

105

110

115

120

125

130